

## UNITED STATES PATENT OFFICE

JOHN V. O. PALM, OF CLEVELAND HEIGHTS, OHIO, ASSIGNOR TO THE CLEVELAND GRAPHITE BRONZE COMPANY, OF CLEVELAND, OHIO, A CORPORATION OF OHIO

## ALLOY

No Drawing.

Application filed September 30, 1926. Serial No. 138,812.

The present invention relating, as indicated, to alloys is particularly directed to a lead babbitt composition having properties and physical characteristics comparable to that of standard babbitt, but costing considerable less to manufacture. A further object of the invention is the provision of a lead babbitt composition having high ductility permitting it to be worked by rolling and otherwise for the purpose of applying it to other metal articles as a surface bearing material, or to be rolled and formed into bearings and similar articles. To the accomplishment of the foregoing and related ends, 15 said invention, then, consists of the means hereinafter fully described and particularly pointed out in the claims.

The following description sets forth in detail one approved combination of ingredients 20 and method of making same embodying my invention, such disclosed ingredients and procedure constituting, however, but one of various forms in which the principle of the invention may be used.

25 My improved composition consists of lead in a predominating amount with smaller amounts of copper, tin, mercury and antimony. In a preferred embodiment of the invention I employ lead in an amount equal 30 to 70 to 75 per cent of the total composition, copper to the extent of 5 or 6 per cent, tin about 12 per cent, mercury about 4 per cent and antimony from 4 to 8 per cent. If a higher ductility is required the amount of 35 antimony is reduced. The above composition is entirely comparable in its physical properties to a standard babbitt and is approximately 50 per cent cheaper to manufacture. It is of course to be understood that the specific 40 proportion of ingredients referred to above may be varied within a reasonable range without departing from the spirit of this invention. It also possesses the important property of not obtaining its full tensile 45 strength and hardness for approximately 24 hours after casting, and it is possible that there is some amalgamating action occurring during this period by reason of the mercury content, which acts to reduce the size of the 50 crystals and gives the same effect as in cast-

ing an ordinary babbitt against a cold mold. In my present composition I first mix copper and tin and to this molten composition add the antimony and subsequently the mercury and lead. For convenience the copper 55 and tin are ordinarily alloyed first, as are the mercury and the lead.

Other modes of applying the principle of my invention may be employed instead of the one explained, change being made as regards 60 the process herein disclosed or the materials employed in carrying out the process, provided the ingredient or ingredients stated by any of the following claims or the equivalent 65 of such ingredient or ingredients be employed.

I therefore particularly point out and distinctly claim as my invention:—

1. A bearing alloy consisting of 70 to 75 per cent of lead, approximately 5 per cent 70 copper, 12 per cent tin, 4 per cent mercury and 4 to 8 per cent of antimony.

2. An alloy consisting of 70 to 75 per cent of lead, 5 to 6 per cent of copper, antimony 75 4 to 8 per cent, mercury approximately 4 per cent and the balance of tin.

Signed by me, this 28th day of September, 1926.

JOHN V. O. PALM.

80

85

90

95

100